

July 22, 1930.

C. D. JOHNSON

1,771,379

METHOD OF COATING WIRE

Filed May 31, 1929



Fig. 1.



Fig. 2.

Inventor.  
Charles D. Johnson  
by Edward Smith & Tennant.  
Atty's.

## UNITED STATES PATENT OFFICE

CHARLES D. JOHNSON, OF WORCESTER, MASSACHUSETTS, ASSIGNOR TO JOHNSON STEEL & WIRE CO. INC., OF WORCESTER, MASSACHUSETTS, A CORPORATION OF MASSACHUSETTS

## METHOD OF COATING WIRE

Application filed May 31, 1929. Serial No. 367,184.

This invention relates to the coating of wire and especially to the application of a coating of copper to wire. One well-known way to coat wire with copper is to pass the wire 5 through a bath of aqueous salt solution such as blue vitriol or a similar coating material. In thus coating the wire it is advantageous to keep the coating bath well agitated so as to maintain it of a uniform consistency. I have 10 discovered that the coating of copper which is deposited on the wire will be heavier and will be applied more evenly when the coating bath is maintained at a relatively low temperature, that is, at a temperature of 40° or 15 50° F., than is the case when the temperature of the coating bath is at a higher temperature, say 70° or 80°.

Because of this fact the coating of copper which is applied to the wire will be heavier 20 and will be more evenly applied when the coating apparatus is started up on a cool day than it will be later in the day, since when the machine is started up the bath will be at the low temperature it has acquired during the 25 night while as the day wears on the temperature of the bath naturally rises.

It is one of the objects of my invention to provide a novel method of and apparatus for 30 coating the wire by which the means for agitating the bath and keeping it thoroughly stirred may be used to maintain the desired low temperature in the bath.

The coating bath is kept agitated by introducing air into it, the air bubbling up through 35 the liquid bath and thus keeping it thoroughly stirred and mixed. In order to provide for maintaining the desired temperature in the bath I propose to cool the air which is admitted to the bath so that the air which agitates 40 the bath will serve also to cool the bath and keep it at the desired cold temperature. This may conveniently be done by providing a cooling chamber which has in it some cooling unit and then by blowing air through the 45 chamber and into the bath, the air becoming sufficiently cool while passing through the chamber to perform the desired function of keeping the bath cool. Another feature of the invention relates to a novel manner of treating 50 the coated wire after it leaves the aqueous

coating bath by which it is thoroughly dried and at the same time polished before it is exposed to the atmosphere for any appreciable length of time. The advantage resulting from this is that the drying can be accomplished with no appreciable oxidization of the 55 wire.

According to this feature of the invention the coated wire as it comes from the washing bath is first subjected to the action of wipers 60 to remove surplus water and then is immediately passed into and through a bed of highly heated granular material such as sand or gravel. The high heat developed quickly evaporates any moisture which remains on the wire thus thoroughly drying it and because of the granular nature of the material it will have a polishing effect on the wire so that the 65 coated wire will come from the heated bed of sand or gravel thoroughly dry and in a polished condition. 70

In order to give an understanding of the invention I have illustrated in the drawings a selected embodiment thereof which will now 75 be described after which the novel features will be pointed out in the appended claims.

In the drawings, Fig. 1 is a diagrammatic view illustrating a coating apparatus embodying my invention;

Fig. 2 is a plan view of the coating bath and 80 the cooling apparatus therefor.

The actual coating of the wire is performed in usual way by passing it through a bath of aqueous coating material, such as blue vitriol if the wire is to be coated with copper. 85

As shown in the drawings the wire to be coated is indicated at 1 and the coating bath is shown at 2, it being contained in a suitable container 3. The wire is shown as being drawn from a spool 4 and as passing through an acid bath 5 and thence through a washing bath 6 in which it is washed and thence through the aqueous coating bath 2. As the coated wire emerges from the aqueous coating bath 2 it passes through another washing bath 7 after which it is passed through a highly heated bed of sand or gravel 8 by which it is thoroughly dried and polished, the coated wire then being wound up on the spool 19. 95

The container 3 for the aqueous coating 100

bath 2 has located in it a coil of pipe 9 which is provided with numerous perforations, so that air which is forced into the pipe 9 will escape through the perforations and bubble up 5 through the bath 2 thus keeping it thoroughly agitated.

The pipe 9 leads to a cooling chamber 10 which is provided with means for cooling the air therein and said chamber is connected by a 10 pipe 11 with a blower or air-forcing mechanism 12.

Any suitable means may be employed in the cooling chamber 10 for cooling the air therein. I have herein shown at 13 a cooling 15 unit which may be any of the well known electrically-actuated units of the type used in electric refrigerators or may be any suitable cooling unit.

In the operation of the device the blower 20 12 blows air into and through the cooling chamber 10, the air passing from the cooling chamber to the pipe 9 from which it is delivered into the coating bath. The size of the 25 cooling chamber 10 and the size of the cooling unit 13 will be such that the air which is delivered from the cooling chamber will be at a relatively low temperature. The air bubbling up through the bath 2 will keep it 30 thoroughly agitated and by having the air delivered to the bath at the proper low temperature, the temperature of the aqueous 35 coating solution will be kept at the proper sub-normal point to ensure the deposit on the wire of an even coating of uniform thickness.

With my apparatus it is possible to maintain the bath 2 at a substantially uniform temperature regardless of weather conditions and thus it is possible to apply to the wire 40 an even coating throughout the day and regardless of changes of temperature in the room. Moreover, I find that the coating which is applied when the bath is at a relatively low temperature adheres to the wire 45 better and is less likely to flake off than a coating which is applied when the bath is at a temperature of 70° F. or 80° F.

After the coated wire leaves the coating bath 2 and passes through a washing bath 7 50 of water by which it is cleaned and as it leaves the washing bath 7 the surplus water is removed therefrom by some suitable means such as the wipers 14. The wire is then immediately passed through a bed 8 of highly 55 heated granular material such as sand or gravel. The high temperature of the sand or gravel quickly evaporates any water or moisture remaining on the coated wire after passing through the wipers and as this drying is 60 done while the wire is embedded in the granular material there will be no appreciable oxidization of the wire as it is dried such as might occur if the wire were dried in the open air because of the fact that the wire is protected 65 from contact with the air by the sand or

gravel. Moreover, the granular material will have a polishing or cleaning effect on the coated wire so that as it leaves the highly heated bed 7 of sand or gravel it will not only be thoroughly dried but will also be more or less polished. 70

The bed 8 of sand or gravel can be heated in any suitable way. As herein shown it is located on the top of a heating chamber 15 which may be heated by any suitable means such as a burner tube 16 for burning oil or gas. With this arrangement the sand 8 can be kept at a relatively high temperature necessary for quickly drying the wire. 75

I claim:

1. The method of making metal-coated wire which consists in passing uncoated wire through an aqueous metal-coating bath whereby it is coated, then passing it through a washing bath whereby it is cleaned, then removing surplus water from it and passing it immediately through a mass of highly heated granular material by which said metal-coated wire is both thoroughly dried and polished prior to substantial contact with the 90 air. 80

2. The method of making metal-coated wire which consists in passing the wire through an acid bath for cleaning it and thence through a water bath for washing it 95 and thence through an aqueous metal-coating bath whereby it is metal coated, then passing the wire through a washing bath whereby it is cleaned, removing the surplus water from the wire as it leaves the washing bath and 100 immediately passing the wire through a mass of highly heated inert granular material whereby the coated wire is dried while buried in the heated granular material and before it is exposed to the atmosphere for any appreciable length of time. 105

3. The method of making metal-coated wire which consists in passing the wire through an aqueous metal coating bath whereby it is metal coated, keeping the bath 110 at a uniform low temperature and simultaneously agitating the bath by introducing into the bath cooled air which bubbles up therethrough whereby a coat of substantially even thickness will be applied to the wire. 115

In testimony whereof, I have signed my name to this specification.

CHARLES D. JOHNSON.

120

125

130